

## UNITED STATES PATENT OFFICE

2,276,346

## DIELECTRIC COMPOSITION

Samuel Ruben, New Rochelle, N. Y.

No Drawing. Application September 8, 1939,  
Serial No. 293,948

8 Claims. (Cl. 106—191)

This invention relates to a composition of matter, particularly plasticized compositions suitable for use as dielectrics and electrical insulating materials.

The general object of the invention is the provision of a new composition of matter suitable for use as a dielectric and as an electrical insulator.

A specific object is the provision of an improved dielectric for electric condensers.

Another object is the provision of an improved dielectric for cables, coils and the like.

Still another object is the provision of a dielectric plasticizer for ethyl cellulose and similar materials.

Other objects will be apparent as the disclosure proceeds.

Ethyl cellulose possesses certain advantages as a dielectric film base material. It is mechanically strong and has high insulation resistance. However, it also possesses certain disadvantages, such as high power factor which, while in the order of 1.3% at normal temperatures, rises to an excessive value when the ethyl cellulose is heated, as when used in an alternating current circuit. This continuous rise in power factor with increase in temperature results in progressive destruction of the ethyl cellulose, especially when it is used as a dielectric in alternating current electrostatic condensers.

Ethyl cellulose requires the use of a plasticizer to render it flexible and to permit the material to withstand mechanical handling. Various plasticizers have been suggested and are now being used, for example, the aromatic esters, but these plasticizers have greater dielectric losses than the ethyl cellulose base and are not electrically as stable.

I have found that the power factor of ethyl cellulose and particularly ethyl cellulose film, is improved considerably by combining the ethyl cellulose with the dimer polymer of di-hydronaphthalene. Also, the addition of the dimer of di-hydronaphthalene provides a permanent plasticizer for the ethyl cellulose and materially improves the resistance of the film to moisture vapor, as well as greatly improving the electrical characteristics. For example, a film can be made utilizing as much as 35% by weight of the dimer of di-hydronaphthalene to the ethyl cellulose and provides a very flexible film and brings about a reduction of the power factor from 1.3% (ethyl cellulose film) to 0.56%. In addition, and of considerable importance, it reduces the rise in power factor with temperature.

The dimer is preferably combined with the ethyl cellulose in a common solvent such as xylol and the film cast from a mixture such as a 20% solution, in the manner well known in the art.

The use of the dimer of di-hydronaphthalene as a film plasticizer appears to be limited to materials with which it is miscible or which have a common solvent. Thus, the di-hydronaphthalene dimer may be combined with polystyrene as mentioned in my prior and copending application Serial No. 285,559, filed 20 July, 1939. In the present invention the dimer of di-hydronaphthalene is combined specifically with ethyl cellulose or benzyl cellulose.

The dimer of di-hydronaphthalene can also be added directly to the cellulose by heating the two materials together. While the materials will combine in practically all proportions the percentage of dimer of di-hydronaphthalene used is dependent upon the desired electrical and mechanical characteristics. For use as a dielectric spacer in an electrostatic condenser, the preferred range is from 5% to 50% dimer of di-hydronaphthalene with a preferred maximum of 35%. Above 50%, the cold flow characteristics of the ethyl cellulose-di-hydronaphthalene dimer composition render the material less desirable as a solid or film spacer, although applicable for other purposes.

One reason why the dimer of di-hydronaphthalene can be used in greater percentages than the commonly used ethyl cellulose plasticizers such as aromatic esters, castor oil and chlorinated hydrocarbons, is that its electrical characteristics are so much superior to that of the ethyl cellulose, that it is advantageous rather than disadvantageous to keep the amount of dimer used at the highest point consistent with good mechanical strength. The dimer of di-hydronaphthalene has a power factor of .02% compared with 1.3% for ethyl cellulose and has a negligible rise of power factor with temperature. It does not oxidize and does not contain catalytically or electrolytically active components as do waxes or acid organic compounds when impregnated into spacers and used in electrostatic condensers at high voltage.

While the improved composition of matter herein described must contain essentially the combination of ethyl cellulose and the dimer of di-hydronaphthalene, the addition of other materials is not excluded. Also, while the specification specifically describes the use of a film of ethyl cellulose-di-hydronaphthalene dimer, it is obvious that the product can be used in other

forms, such as lacquers, cast solids, etc., depending upon the proportions used and the amount of added solvents.

Other polymers of di-hydronephthalene such as the tetramer will also combine with ethyl cellulose but in general such compositions are not as satisfactory as the combination of the dimer of di-hydronephthalene with ethyl cellulose.

What is claimed is:

1. A composition of matter comprising a cellulose derivative of the class consisting of ethyl cellulose and benzyl cellulose and dimer of di-hydronephthalene.

2. A dielectric comprising a cellulose derivative of the class consisting of ethyl cellulose and benzyl cellulose and dimer of di-hydronephthalene.

3. A composition of matter comprising a film of a cellulose derivative of the class consisting

of ethyl cellulose and benzyl cellulose and dimer of di-hydronephthalene.

4. A composition of matter comprising a cellulose derivative of the class consisting of ethyl cellulose and benzyl cellulose, dimer of di-hydronephthalene and a common solvent.

5. A composition of matter comprising dimer of di-hydronephthalene 5% to 50% and ethyl cellulose 50% to 95%.

10 6. A composition of matter comprising a cellulose derivative of the class consisting of ethyl cellulose and benzyl cellulose and a polymer of di-hydronephthalene.

7. A composition of matter comprising ethyl cellulose and dimer of di-hydronephthalene.

15 8. A dielectric for electric condensers, cables, coils and the like comprising ethyl cellulose and dimer of di-hydronephthalene.

SAMUEL RUBEN.